

## UNITED STATES PATENT OFFICE

2,082,371

## PROCESS FOR MANUFACTURE OF MISCELLANEOUS GUM FROM DRYING OILS

Edward M. Williams, Elyria, Ohio

No Drawing. Application October 16, 1933,  
Serial No. 693,834

6 Claims. (CL. 87—12)

My invention relates to gum compounds of the miscible type, and to processes of making the same.

It relates more particularly to a vegetable oil miscible gum compound wherein the vegetable oils are so processed to a miscible gum that the characteristics of the said oils are changed.

It is an object of my invention to pre-oxidize vegetable oils in processing the same to a gum, so that paint film produced from the gum resists further oxidation.

It is another object of my invention to so process vegetable oils to a miscible gum as to reduce the film shrinkage of the resultant gum to a minimum, and also to build up the oils to better resist oxidation.

Another object of my invention is to provide a miscible gum from vegetable oils and chemicals which will reduce with paint solvents such as mineral spirits, naphtha, and turpentine, and be adaptable to the make-up of paints, varnishes, japsans, and enamels.

Another object of my invention is to provide a miscible gum which, when reduced with solvents such as mineral spirits, naphtha, or turpentine, will have a valve action in regard to moisture so as to provide a protective coating for steel and iron.

Another object of my invention is to provide a miscible gum which will withstand unusual reduction with solvents such as mineral spirits, naphtha, and turpentine, and maintain good body.

Another object of my invention is to provide a gum which will incorporate with vegetable oils, rosin, ester gum, synthetic resins, natural resins, asphalts, and pigments.

Another object of my invention is to provide a miscible gum of the type described which is inexpensive to process and economical and enduring in use.

Other objects of my invention and the invention itself will become apparent by reference to the following description of the invention and process of making the same.

In producing my improved gum, I first charge a quantity of menhaden fish oil with a lesser quantity of China-wood oil, in a suitable kettle or tank. I then heat the oil to a temperature of approximately 400° Fahrenheit, and at this temperature blow enough air into the bath to produce a mild agitation therein, and to accelerate oxidation. The amount of pressure required will naturally vary depending upon the volume of the charge. Necessarily, more pres-

sure will be required if the charge is great than if it is small. Also a narrow kettle or tank will require more pressure than a wide shallow one for the same gallonage.

Better results and a more uniform product will be produced by enclosing the top of the kettle or tank. A suction fan or other means may be employed to draw off the mist arising from the bath, and also to permit re-claiming any by-product, mainly fatty acids and glycerides arising therefrom. The latter are extracted to aid in reducing film shrinkage and in building up resistance in the resultant product.

At the temperature of approximately 400° Fahrenheit, I then add sufficient lead acetate and cobalt acetate to hasten oxidation. The cobalt and lead driers act as catalytic agents conducting the oxygen from the air to the oil.

The following figures indicate the relative proportions used in the process, but the exact figures are not to be taken as an essential part of this invention:

|                | Pounds |
|----------------|--------|
| Menhaden       | 3836   |
| China-wood oil | 425    |
| Lead acetate   | 19     |
| Cobalt acetate | 8      |

Processing the above charge at a temperature of about 400° Fahrenheit, approximately forty-eight hours with sufficient air to produce a slight agitation in the bath and a suction fan to draw off the mist, reduces the charge to a heavy bodied oil.

The temperature range, it should be noted, can vary considerably. If it is desired to operate the process above 400° Fahrenheit, undoubtedly the time of processing would be reduced and the time of drying or curing of the vehicle increased. A lower temperature than 400° Fahrenheit undoubtedly would increase the time of processing and reduce the drying or curing time of the vehicle produced from the gum.

It is also to be noted that China-wood oil and menhaden are merely the preferred oils used in this process. It is possible to substitute perilla oil for the China-wood oil, and to substitute other fish oils for menhaden. Likewise, any suitable metallic drier might be used in place of the cobalt and lead acetates.

After the aforesaid process is completed, the heavy bodied oil or gum produced thereby is then charged with a quantity of linseed oil and China-wood oil in a varnish kettle or tank, preferably covered, to permit the carrying off of

fumes with a suction fan or other means. This mixture is then heated to approximately 400° Fahrenheit, and a small amount of cobalt acetate, lead acetate, and calcined magnesium oxide added at this temperature.

The bath is then blown with sufficient air to produce agitation therein, and, as in the case of the first process, to aid oxidation.

If desired, in making a gum suitable for certain varnishes, paints, or enamels, the proportionate amount of linseed oil used in this process could be increased to increase the iodine content of the resultant gum. The calcined magnesium oxide added is used to build up a good body and also to produce a body which can be readily reduced with the lower grades of solvents, such as kerosene and mineral spirits.

The following figures are given to illustrate the respective quantities of the various ingredients used in the second process, in order to indicate the relative proportions used, but the exact figures are not to be taken as essential to this invention:

|    |                                            |         |     |
|----|--------------------------------------------|---------|-----|
| 25 | Raw linseed oil                            | gallons | 50  |
|    | China-wood oil                             | do      | 12½ |
| 30 | Heavy bodied oil produced by first process | gallons | 25  |
|    | Lead acetate                               | pounds  | 3   |
|    | Cobalt acetate                             | do      | ¾   |
|    | Calcined magnesium oxide                   | do      | 19  |

This second process runs at a temperature of approximately 400° Fahrenheit, and also requires approximately forty-eight hours to complete under the same method of operation as for the first process. A higher temperature will undoubtedly shorten the time, while a lower temperature would increase the time necessary to complete the gum.

40 The gum produced by the several processes is then reduced or "cut" with kerosene, turpentine, mineral spirits, naphtha, or other paint cutters, and can be reduced to a liquid with the higher solvents cold with agitation. It can also be reduced by heating the gum to a temperature around 400° Fahrenheit or up to 550° Fahrenheit, at which temperature it will readily cut with the solvents mentioned without any prolonged heating. A higher temperature than 400° Fahrenheit is not necessary and increases the fire hazard.

45 It is to be noted that the gum produced by the several processes described above will withstand unusual reduction with low solvents, such as kerosene and mineral spirits, and maintain good body. For example, eight pounds of the miscible gum produced by the several processes can be reduced with two and one-half gallons of mineral spirits, kerosene, naphtha, or turpentine, and maintain a viscosity of between F and G on 50 Gardiner-Holt viscosity tubes. Few gums or resins withstand more than a reduction of equal parts by volume and maintain a viscosity of A on this viscosimeter. A gallon of the miscible gum produced by the several processes weighs approximately eight pounds.

55 The improved gum of my invention when reduced to a liquid by the addition of any of the cutters referred to, produces a film with no appreciable shrinkage during drying or curing.

60 It should be noted in this connection that the shrinkage of a paint film in drying depends almost entirely upon the vehicle used, which in most paints is composed of vegetable oils. Linseed, one of the most extensively used oil, when reduced to a paint film, shrinks in volume some-

times as much as twenty to thirty percent even though at the same time it gains twenty to twenty-five percent in weight from oxygen with which it combines chemically. As the state of oxidation increases, the elongation of the linseed film decreases.

65 This rapid oxidation of the linseed film and its corresponding decrease in elongation reduce its value for the protection of steel and iron, since the coefficient of expansion and contraction of steel and iron is constant. After a given stage of oxidation, a paint carrying raw or boiled linseed oil loses the elongation necessary to provide for the expansion and contraction of steel and iron, which is inevitable upon the change of 15 temperature. The movement in the steel or iron thus causes cracks in the paint film through which atmosphere and moisture, the common causes of rust, are admitted into contact with the unprotected metal. All of the vegetable oils, 20 China-wood oil, perilla oil, soya bean oil, and fish oil have similar characteristics to linseed.

25 By changing the characteristics of the oils used as to drying or curing during processing, as I have done, it is apparent that while the vegetable oils used in the process in their raw or boiled state have considerable shrinkage as explained, the oils produced by cutting the gum are pre-oxidized and drying is started by the evaporation of the cutter similar to the setting up of 30 lacquer. After the evaporation of the cutter, surface oxidation sets in, but since the oils have been pre-oxidized they naturally will not absorb any great amount of oxygen.

35 The elimination of shrinkage by my invention thus is a distinct improvement in a paint film, particularly in a paint film used on steel and iron. It can also be used to advantage in baking japans and enamels since the bond of the enamel to the steel or other surface is better as the shrinkage 40 is decreased.

45 Another important advantage of the gum of my invention is that when it is reduced with paint cutters, such as are referred to above, applied and given a reasonable period to cure, it is highly resistant to diluents such as mineral spirits, kerosene, gasoline, transformer oils, lubricating oils, cottonseed oil, and Pennsylvania crude oil.

50 The fact that the gum will readily reduce in the form of gum with paint cutters, and when reduced to a film and given sufficient time to cure, will not only not reduce, but will provide a protection against such reducers, is sufficient proof of surface oxidation and indicates that a chemical reduction takes place in curing.

55 The film, it is evident, may be used, therefore, for coating the inside of gasoline tanks and tanks carrying the other liquids mentioned, viz., kerosene, transformer oils, lubricating oils, etc.

60 The gum produced by the several processes, described above, may also be cut so as to make it a good vehicle for calorizing aluminum to steel. For this purpose, the gum should preferably be reduced in a ratio of approximately eight pounds or one gallon of gum with five gallons of mineral spirits. To the vehicle produced thereby, two pounds of aluminum powder per gallon should be added. Various other quantities of gum, solvent, and aluminum in such relative proportions might also be used. The steel or iron parts to be coated must be thoroughly cleaned from mill scale, rust, and other foreign matter. The aluminum paint should preferably then be applied to such parts 70 75

with a spray gun, although it could be applied by brushing or dipping.

Approximately twenty to thirty minutes should be allowed for the aluminum paint to air dry after it is applied to the steel or iron parts, which are at that time put into an oven at a temperature of around 250° Fahrenheit. The temperature of the oven should now be brought slowly to approximately 1100° Fahrenheit. The process described 10 will calorize aluminum to steel, and after such calorization, the aluminum will withstand high temperatures; for example, it will stand 400 to 500 degrees more than galvanized sheet steel. This is very desirable in a coating of steel which 15 will be subjected to high temperatures, such as boiler fronts, stove pipes connecting a furnace to a chimney, and the like.

The heavy bodied oil or gum produced by the first process may be used in an advantageous 20 manner for various purposes without subjecting the same to the second process. It may be used for producing valve action vehicles, preferably for coating steel. It may be used as an emulsion for coating porous surfaces such as rough plaster, 25 porous concrete, insulating board, paper, and other porous surfaces to build up a base for paint. It may also be used for preventing efflorescence on brick.

The oil produced by the first process, when reduced with mineral spirits in a proportion of 30 equal parts of gum and mineral spirits, as a gallon of gum, weighing approximately eight pounds, with a gallon of mineral spirits, shows a valve action in regard to moisture so as to provide a better coating for the protection of steel and iron. As is well known, a large tonnage of steel rusts before fabricated and coated. Bridges, tanks, fire 35 escapes, and other steel structures are subject to such deterioration.

40 On repaint jobs, this rust must be removed unless the paint vehicles are especially processed as described, to penetrate through the rust to the unoxidized surface beneath and seal the unoxidized surface against atmosphere and moisture. As rust contains approximately twenty-two percent of moisture by weight, to remove this moisture content and stop the rust at its present stage, it is essential that a valve action vehicle be used 45 that will absorb the moisture content of rust and 50 pass it through the film by evaporation.

Taking the heavy bodied oil which is produced by the first process of forty-eight hours, and cutting it with equal parts of mineral spirits, produces a paint vehicle which has maximum penetrating qualities. When it is applied over rust it penetrates through the rust to the unoxidized surface beneath, sealing this surface against atmosphere and moisture, and combines with the moisture content in the rust and passes through 60 the film by evaporation, stopping the rust action at its present stage. After the cutter evaporates, surface oxidation sets in and this surface oxidation prevents moisture from entering from the outer surface.

65 To produce a good emulsion from the heavy bodied oil or gum of the first process, to be used as a prime coat on porous surfaces and the like, to build up a base for finishing coats, the following procedure may be used. Heat a quantity of the 70 gum to just under the boiling point of water; to this add a quantity of tap water at the same temperature; agitate the mass quite violently and to this mixture add a greater quantity of water containing sufficient ammonia to make it alkaline.

The following proportions are given to indicate the relative proportions which should be used:

2 lbs. of gum  
1/2 pt. of tap water  
3 half-pts. of water containing a small amount 5 of ammonia.

In order to agitate the mixture violently enough, the agitation should be produced by mechanical means. The proportions given above provide a good brushing consistency.

10 To produce a vehicle which will prevent efflorescence on brick, I preferably use one pint of the heavy bodied oil or gum of the first process with one and one-half pints of mineral spirits, naphtha, turpentine, or any good paint cutter. For example, eight pounds of gum could be cut with one and one-half gallons of mineral spirits, mineral spirits being preferable since it is lower in cost than most solvents.

15 Particularly it should be noted that the gum produced by the joint processes described herein withstands unusual reduction. This can be attributed to a great extent to the processing with calcined magnesium oxide. It is to be noted that the gum of the first process will withstand a possible reduction of one gallon of gum to one gallon of mineral spirits, while the gum produced by the joint processes withstands a reduction of one gallon of gum to two and one-half gallons of mineral spirits to produce the same viscosity.

20 Although I have described my invention in specific embodiments, I am aware that numerous and extensive departures involving equivalency, 25 may be made from my improved gum compound as above described, and I therefore claim my invention broadly as defined in the accompanying claims.

I claim:

1. A process for the production of a miscible 30 gum which comprises heating a quantity of China-wood oil with a greater quantity of menhaden oil at a temperature of approximately 400° Fahrenheit, adding a quantity of lead acetate, and cobalt acetate at said temperature, and aerating the mixture to produce a thickened oil 45 mixture, adding a quantity of linseed oil and China-wood oil, to said heavy bodied oil, heating the same at a temperature of approximately 400° Fahrenheit, adding up to five percent by weight of lead acetate, cobalt acetate, and calcined magnesium oxide at such temperature, and processing the same to a gum.

2. A process for the production of a miscible 50 gum which comprises heating a quantity of China-wood oil with a greater quantity of menhaden oil at a temperature of approximately 400° Fahrenheit, adding a quantity of lead acetate, and cobalt acetate at said temperature, and aerating the mixture and processing the same for approximately forty-eight hours to produce a thickened oil 55 mixture, adding a quantity of linseed oil and China-wood oil, to said mixture, heating the same at a temperature of approximately 400° Fahrenheit, adding up to five percent by weight of lead acetate, cobalt acetate, and calcined magnesium oxide at such temperature, and further processing the same to a gum for approximately forty-eight hours.

3. A process for the production of a miscible 60 gum which comprises heating a quantity of China-wood oil with a greater quantity of menhaden oil at a temperature of approximately 400° Fahrenheit, adding a quantity of lead acetate, and cobalt acetate at said temperature, and aerating the mixture to produce a thickened oil 65

70

mixture, and drawing off the fatty acids and glycerides arising from the bath, adding a quantity of linseed oil and China-wood oil, to said mixture, heating the same at a temperature of approximately 400° Fahrenheit, adding up to five percent by weight of lead acetate, cobalt acetate, and calcined magnesium oxide at such temperature, and processing the same to a gum.

4. A process for the production of a miscible gum which comprises heating a quantity of a drying vegetable oil having the drying characteristics of the class consisting of China-wood and perilla oils with a greater quantity of fish oil at a temperature of approximately 400° Fahrenheit, adding a quantity of lead acetate, and cobalt acetate at said temperature, and aerating the mixture to produce a thickened oil mixture, adding a quantity of linseed oil and a drying vegetable oil having the drying characteristics of the class consisting of China-wood and perilla oils, to said heavy bodied oil, heating the same at a temperature of approximately 400° Fahrenheit, adding up to five percent by weight of lead acetate, cobalt acetate, and calcined magnesium oxide at such temperature, and processing the same to a gum.

5. A process for the production of a miscible gum which comprises heating a quantity of a drying vegetable oil having the drying characteristics of the class consisting of China-wood and perilla oils with a greater quantity of fish oil at a temperature of approximately 400° Fahrenheit, adding a quantity of lead acetate, and cobalt acetate at said temperature, and aerating the mix-

ture and process the same for approximately forty-eight hours to produce a thickened oil mixture, adding a quantity of linseed oil and a drying vegetable oil having the drying characteristics of the class consisting of China-wood and perilla oils, to said mixture, heating the same at a temperature of approximately 400° Fahrenheit, adding up to five percent by weight of lead acetate, cobalt acetate, and calcined magnesium oxide at such temperature, and further processing the same to a gum for approximately forty-eight hours.

6. A process for the production of a miscible gum which comprises heating a quantity of a drying vegetable oil having the drying characteristics of the class consisting of China-wood and perilla oils, with a greater quantity of fish oil at a temperature of approximately 400° Fahrenheit, adding a quantity of lead acetate, and cobalt acetate at said temperature, and aerating the mixture to produce a thickened oil mixture, and drawing off the fatty acids and glycerides arising from the bath, adding a quantity of linseed oil and a drying vegetable oil having the drying characteristics of the class consisting of China-wood and perilla oils, to said mixture, heating the same at a temperature of approximately 400° Fahrenheit, adding up to five percent by weight of lead acetate, cobalt acetate, and calcined magnesium oxide at such temperature, and processing the same to a gum.

EDWARD M. WILLIAMS.